

# UNITED STATES PATENT OFFICE.

ANSON GARDNER BETTS, OF TROY, NEW YORK.

## TREATING ANODE SLIME FROM THE ELECTROLYTIC REFINING OF LEAD.

No. 918,647.

Specification of Letters Patent.

Patented April 20, 1909.

Application filed January 23, 1907. Serial No. 353,641.

To all whom it may concern:

Be it known that I, ANSON GARDNER BETTS, a citizen of the United States, residing at Troy, in the county of Rensselaer and State of New York, have invented certain new and useful Improvements in Treating Anode Slime from the Electrolytic Refining of Lead, of which the following is a specification.

10 This invention relates to processes of taking metals into solution from the slime without previous drying or fusion.

Hitherto slime produced in electrolytic lead refineries has been always collected with considerable trouble, and washed to recover the lead depositing electrolyte contained in it, before being submitted to chemical or metallurgical treatment, and even then there is a loss of lead-depositing electrolyte.

20 Some objects of my invention are to save the expense in collecting and washing the slime, and at the same time to provide a simpler and more rational treatment than those existing at present.

25 Other objects will appear in connection with the following description.

I have discovered that I can dissolve both the antimony and lead in the slime, as well as copper, silver and arsenic if desired, by the use of a solution containing an acid making a soluble lead salt, *e. g.* fluosilicic acid and also hydrofluoric acid in moderate quantity.

30 A solution of lead fluosilicate and fluosilicic acid containing 5-6% lead and 15%  $\text{SiF}_6$  ion I have discovered permits the addition to it of as much as 5% anhydrous HF at a moderate temperature, and considerably more at an elevated temperature. Such a solution containing 5% HF is capable of dis-

35 solving 10% antimony as trifluorid, and I have further discovered that a solution of antimony trifluorid even in large proportions will not precipitate lead fluorid from a lead solution, as the addition of most fluorids, for example, sodium fluorid, will do. I prefer to use, then, to take the metals of the slime into solution a liquid containing considerable fluosilicic acid, and a moderate quantity of hydrofluoric acid.

40 50 I have discovered that lead peroxid used in connection with fluosilicic or other equivalent acid will not only cause metallic lead, copper, etc., to go into solution as fluosilicates, etc., but will also cause antimony to go

into solution as fluorid, if hydrofluoric acid is present in a moderate proportion.

As the solution becomes more neutral, the precipitating power for lead of the hydrofluoric acid becomes greater, from the increasing proportion of lead to be precipitated and the decreasing proportion of fluosilicic acid remaining to tend to dissolve any lead fluorid formed. However, the proportion of hydrofluoric acid becomes less, as antimony trifluorid is being formed, so no lead fluorid is precipitated. Similar changes take place in a reverse direction in the preferred method of electrolyzing the solution, described below.

Lead peroxid is a powerful oxidizing agent, sufficiently so to cause the formation of silver salts from metallic silver, so I am able to dissolve practically all of such metals of the slime as copper, lead, antimony, tin, silver, and certain amounts of bismuth. However, lead peroxid, especially in the form in which I prefer to produce it, is a slow oxidizing agent, so I prefer to grind it fine before use, and I believe the presence of traces of chromium in the solution act as a catalytic agent and hasten the reaction.

55 In the practical execution of my process I prefer to proceed as follows: The lead anodes are suspended in a tank in the usual way with the usual cathodes, and the whole electrolyzed until the anodes are pretty well dissolved. By suitable means, before or after siphoning the clear solution out of the tank, I cause the slime to drop from the anodes to the bottom of the tank. After removing anode scrap, I then add about the theoretical amount of lead peroxid, necessary to carry out the following reactions:



The reactions with bismuth and tin are of minor importance as these elements are

usually entirely absent or occur in relatively small quantities. The reactions given are those which I suppose to take place.

- The tank is nearly filled with strong  $H_2SiF_6$  solution containing some lead which may have the composition  $SiF_6$  ion 20%, lead 3-4%, HF 1 to 2% and stirred preferably until solution is practically complete, or until the slime gets so thin from the 5 solution of its antimony, that it can readily be drawn off, which it is difficult to do with most raw slimes, on account of their heavy nature. The tank is finally cleaned out, and used to refine more lead.
- 10 After action is practically complete, the solution, which may contain about 2% antimony, 0.6% arsenic, 1% silver, 1% copper, 18% lead and perhaps 0.1% bismuth, the figures of course subject to great variation, 15 is filtered from gold, and undissolved silver and lead peroxid. The residue is so small in quantity that the loss of fluosilicic acid not washed out is much reduced from the present practice.
- 20 I prefer the use of tanks of concrete or cement treated with sulfur as described and claimed in my United States application, Serial Number 346678, filed December 6th, 1906, as being easier to clean and allowing 25 no absorption of solution containing metals, to afterward diffuse out and render impure lead subsequently deposited in the tank. If the usual wooden tanks are in use, it will be better to remove the slime to special 30 slime treatment tanks, before treatment.

The solution containing the various metals of the slime is led through tanks in which are suspended copper plates, to precipitate out metallic silver. It then passes through a 40 series of electrolytic tanks provided with carbon anodes and suitable cathodes, copper being good for some or all and lead for others, in which a current density is used varying from 5 to 10 or more amperes per square foot 45 with an electromotive force of from 2.2 to 2.5 volts per cell.

Electrolytic copper is deposited on the first cathodes, and continues to deposit until copper is reduced to say 0.1 to 0.2%, when a 50 solid alloy of copper and antimony deposits further on in the series of cells, and then impure lead, and then fairly pure lead.

I have found lead peroxid to deposit on the anodes throughout, so that only one anode 55 product is obtained, which is ground and returned to be used in slime treatment.

The cathode deposits are better than expected and are quite satisfactory mechanically. The impure cathodes I prefer to work 60 up by using them as anodes in a refinery cell, in a series of tanks through which the solution from the slime treatment passes. For example, the copper-antimony cathodes are used as anode and refined by the solution as it comes from the silver precipitation, cop-

per and antimony going into solution together, while pure copper deposits. In this way a certain amount of these cathodes are always on hand, but do not accumulate faster than they are worked up.

The lead peroxid precipitates as a very hard, smooth conducting coating which warps slightly and drops off the anodes occasionally, or can be easily split off.

More solution is obtained than was started 75 with, as the slime contained some to start with. Part of the solution should be partially neutralized by treatment with lead peroxid and lead according to the reaction



and after being passed through as special electrolytic lead refining cell with lead anodes and cathodes, for the sake of removing any traces of impurities, passed back to the lead 85 depositing plant.

I may very well also, in treating the slime, use the lead refining solution already in the tank, that is the regular lead refining solution, for dissolving the metals, provided a 90 certain amount of HF is contained therein or added.

I am not limited to the use of lead peroxid as oxidizing agent. I can also use for instance, ferric fluosilicate, which, however, 95 does not appear to dissolve silver much in the cold, and other oxidizing salts. The use of lead peroxid, however, is preferred as not involving the use of a diaphragm in the electrolytic cells, and still giving a high current 100 efficiency, and being simpler in other respects.

By the term "containing fluorin ion", I mean that the solution contains fluorin in condition which shows the ordinary reaction 105 of fluorin. Thus solutions containing hydrofluoric acid or ammonium fluorid, show the reactions of fluorin; for example, they will precipitate insoluble fluorids, as lead fluorid, if the conditions of the test are right, while 110 pure fluosilicic acid solution does not contain appreciable quantities of fluorin ion and will not show the tests for fluorin ion. My usage of the term ion is in accord with that of such standard books as Ostwald's *Principles of 115 Inorganic Chemistry*.

What I claim as new and desire to secure by Letters Patent is:

1. The process of treating anode slime from the electrolytic refining of lead which 120 consists in dissolving metal therefrom by treatment with a solution containing fluorin ion, and with an oxidizing agent, of which the products of reduction by the slime are soluble in the solution, the said solution also containing a strong acid forming a soluble lead salt; and recovering metal of the slime from the resulting solution.

2. The process of treating anode slime from the electrolytic refining of lead which 125

consists in dissolving metal therefrom by treatment with a solution containing fluorin ion, and with an oxidizing agent, the said solution also containing relatively strong acid 5 forming a soluble lead salt, and recovering metal of the slime from the resulting solution.

3. The process of treating anode slime from the electrolytic refining of lead which consists in dissolving metal therefrom by 10 treatment with a solution containing a considerable amount of the same acid as is contained in the electrolyte for refining the lead from which said slime is produced, said solution also containing fluorin ion, and an oxidizing agent, and recovering metal of the 15 slime from the said solution.

4. The process of treating anode slime from the electrolytic refining of lead which consists in dissolving metal therefrom by 20 treatment with lead peroxid and a solution containing fluorin ion and an acid forming a readily-soluble lead salt, and electrolytically recovering lead peroxid and metal of the slime from the resulting solution.

25 5. The process of treating anode slime from the electrolytic refining of lead contain-

ing antimony and copper, which consists in dissolving metal therefrom by treatment with lead peroxid and a solution containing fluorin ion and an acid forming a readily-soluble lead salt, and electrolytically depositing antimony from the solution by electrolysis with an insoluble anode and suitable cathode.

6. The process of treating anode slime 25 from the electrolytic refining of lead containing antimony and copper which consists in dissolving metal therefrom by treatment with lead peroxid and a solution containing fluorin ion and an acid forming a readily- 40 soluble lead salt and electrolytically depositing copper, antimony and lead successively from the solution, by electrolysis with insoluble anodes, simultaneously depositing lead peroxid on the anodes.

In testimony whereof I have signed my name to this specification in the presence of two subscribing witnesses.

ANSON GARDNER BETTS.

Witnesses:

SARA A. MALLORY,  
ETHEL K. BETTS.